

# UNITED STATES PATENT OFFICE.

MADISON L. WOODBURY, OF ST. ALBANS, VERMONT.

## COMPOUND PACKING FOR HOT JOURNALS ON CARS, &c.

SPECIFICATION forming part of Letters Patent No. 280,277, dated June 26, 1883.

Application filed April 4, 1883. (No specimens.)

*To all whom it may concern:*

Be it known that I, MADISON L. WOODBURY, a citizen of the United States, residing at St. Albans, in the county of Franklin, State of Vermont, have invented a new and useful Composition of Matter to be Used for Cooling Hot Journals (sometimes called "hot-boxes") on Cars and Locomotive-Engines, of which the following is a specification.

10 My composition consists of the following ingredients, combined in the proportions stated, viz: talc, (or soapstone,) two hundred pounds; tallow, one hundred pounds; sulphur, twenty-five pounds; lard, five gallons.

15 In making the above-named compound, put in the tallow and heat it hot; then put in the sulphur and keep stirring it until thoroughly dissolved; then put in the lard and stir it until mixed. Keep stirring while the talc or 20 soapstone is being put in. When the whole is thoroughly mixed, let the compound cool.

In using the compound, put it into the box around the heated journal, when the car can be put in motion and the journal will cool 25 while the car or engine is moving, whether at a slow or a rapid rate.

By the use of the above compound all delay on account of hot-boxes is entirely avoided,

and the box will cool while the train is in motion.

30

I am aware that compounds are in use containing one or more of my ingredients.

I am also aware that a composition containing mineral oil, tallow, plumbago, rock-salt, palm-oil, flowers of sulphur, and soapstone has 35 been patented, and I disclaim it. I consider the plumbago, salt, and palm-oil not only useless, but also injurious, in a preparation for cooling a hot-box when the car is in motion; nor could this compound be applied directly 40 to a hot-box and accomplish the result mine does, but the train would have to stop until the box had partially cooled, to say the least.

I am not aware that all of the ingredients of my composition in the proportions stated have 45 been used together.

What I claim, and desire to secure by Letters Patent of the United States, is—

The herein-described compound packing for cooling hot journals, consisting of talc, tallow, 50 sulphur, and lard, in the proportions specified.

MADISON L. WOODBURY.

Witnesses:

NATHAN N. POST,  
M. H. ALEXANDER.